# EUROPEAN PATENT SPECIFICATION

(11) **EP 0 922 918 B1**
(45) Date of publication and mention of the grant of the patent: **04.07.2001**
(21) Application number: 98660057.5
(22) Date of filing: 03.08.1998
(51) Int. Cl.: F26B 21/10, B27K 5/00

(54) **Method for heat treatment of timber**
Verfahren zur Wärmebehandlung von Holz
Procédé de traitement thermique du bois

(30) Priority: 09.12.1997 FI 974468
(43) Date of publication of application: 16.06.1999
(73) Proprietor: Stellac Oy, 50100 Mikkeli (FI)
(72) Inventor: Lallukka, Tero, c/o Stellac Oy, 50100 Mikkeli (FI)
(74) Representative: Helino, Timo Kalervo

(56) References cited:
- WO-A-94/27102
- WO-A-95/31680
- WO-A-98/04392
- WO-A-98/25742
- US-A- 4 182 048
- US-A- 5 678 324
- US-E- R E28 020

## Description

The present invention relates to a procedure for heat treatment of timber, as defined in the preamble of claim 1. Such a procedure is known, for example, from WO-A-95/31680.

International patent application WO-A-94/27102 presents a procedure for improving the resistance to biological decay and the dimensional stability of timber via heat treatment. The specification presents a procedure for the drying of timber at a raised temperature. The procedure aims at ensuring that no cracks are formed in the product. According to the specification, this is achieved by continuously determining the temperatures in the interior parts of the timber and on its exterior surface and continuously maintaining a reasonably small difference between the temperatures. This principle is applied both when the temperature is being raised and when it is being lowered during the drying process. After this, according to the specification, the temperature of the timber is raised rapidly to a level of over 150 °C, and the treatment is continued at this temperature to achieve the desired treatment result.

By the method described, certain properties of timber can be improved, but it has been established that the final result is not exactly homogeneous, in other words, material portions at different depths in the timber undergo somewhat different treatment.

The object of the present invention is to eliminate the drawbacks described above. A specific object of the present invention is to present a new type of procedure for heat treatment of timber, which makes it possible to produce timber that has a very homogeneous and good quality throughout its thickness.

As for the features characteristic of the invention, reference is made to claim 1.

In analysing heat treatment and the changes occurring in the structure of wood and in the substances contained in it, it has unexpectedly been discovered that the way in which the temperature of the wood is raised to the temperature required for the heat treatment and the way in which it is lowered are equally essential in actual heat treatment of timber as the regulation of temperature is in drying. It has been found that timber behaves differently at different temperatures, its structures undergc different changes at different temperatures and its constituents undergo different changes and chemical reactions at different temperatures, and that the duration of action of the temperature is just as decisive for many changes as the level of the temperature.

Therefore, in the procedure of the invention, the timber is first dried to a suitable humidity level below 15 %, whereupon the temperature of the timber is raised above a heat treatment threshold and maintained at the required level for as long as is necessary for the treatment. Finally, the temperature of the timber is lowered below the heat treatment threshold. Heat treatment threshold means the temperature above which the desired changes produced by the heat treatment begin to appear. It is generally about 140 - 150 °C. Furthermore, above the heat treatment threshold, both when the temperature is being raised and when it is being lowered, the difference between the internal and external temperatures of the timber is kept within certain limits. The limit is preferably 10 - 30 °C, e.g. about 20 °C.

According to the invention, the heating and cooling phases above the heat treatment threshold are of equal duration and, in addition, the absolute value of the difference between the internal and external temperatures is maintained at a substantially equal magnitude at temperatures corresponding to each other during heating and cooling. Therefore, practically every part of the timber is at the same temperature, i.e. subject to the same kind of chemical and structural changes in the timber, for a substantially equal length of time. Thus, the heating and cooling processes of the timber are rendered about identical, i.e. mirror image processes above the heat treatment threshold.

In this context, external temperature of timber means the temperature of the air surrounding the timber, which is substantially the same as the surface temperature of the timber, and internal temperature means the temperature in the central part of the timber.

In a preferred embodiment of the invention, both the internal and external temperatures of the timber are raised and lowered in a linear fashion. Likewise, preferably a constant temperature difference is maintained for a substantial part of the time during which the temperature is being raised or lowered.

In a preferred embodiment of the invention, the temperature difference is changed as a function of temperature. In this case, when the temperature is high, the temperature difference is maintained at a low value, e.g. between 5-20°C, and when the temperature is lower, the difference can be increased, e.g. to a value within the range 20-40°C.

Before the heat treatment, the timber should in any case be dried to a humidity below 15 %, but preferably the timber is dried to a humidity below 10, even below 5 %.

The heat treatment threshold, above which the timber begins to undergo changes due to heat, is about 140-150°C, but the high limit of heat treatment may vary considerably depending on the kind and size of the timber and the changes intended to be produced in it. If the aim is to increase the strength, surface hardness, flexural resistance and elastic flexural strength of the timber, the maximum temperature may be 150-200°C, depending on the case. On the other hand, if the main objective of the heat treatment is to improve the rot-proof properties of the timber, the temperature of the timber should be raised to a value between 200 - 300 °C. Further objectives in both of the above-mentioned temperature ranges may be to reduce the propensity of the timber to expand and contract due to humidity, to retard the absorption of water and to change the colour of the wood.

The heat treatment is preferably carried out in a substantially non-pressurised room, in other words, the treatment room may preferably have an overpressure of max. 0.1 bar. Whereas in prior art it has been common to use a high pressure, e.g. about 10 bar, to prevent cracking of the wood, the procedure of the invention uses a controlled and steady treatment, so that no overpressure is needed but the timber endures the treatment at normal pressure without cracking. Therefore, the structures of the treatment chamber can be built e.g. only from thin and light boards, whereas prior-art structures need to have pressure-resistant frameworks and wall surfaces.

As compared with prior art, the procedure of the invention has significant advantages. In the invention, the real behaviour of wood during heat treatment has been clarified, and from timber subjected to heat treatment by the method of the invention it is possible to produce timber material of very homogeneous quality, having the desired properties uniformly throughout its thickness. This has not been possible in any method known so far.

In the following, the invention will be described in detail by referring to the attached drawing, which is graphical illustration of the process stages of the procedure of the invention.

The drawing shows the external temperature Tₒ and the internal temperature Tᵢ of the timber as functions of time.

At instant t₁, when the heat treatment begins, the timber has been dried in a suitable temperature e.g. to a humidity of 5% and it has a roughly uniform temperature, about 140 °C. At this point, the surrounding air is subjected to intensive heating, producing an initial impulse S that gives the process a fast start. The temperature increase is stopped at 180 °C at instant t₂ and the internal temperature Tᵢ is allowed to rise. It begins to rise steadily and at instant t₃ the difference ΔT between the internal and external temperatures is at the desired value, about 20 °C, and at this point the raising of the external temperature is continued. From this point onwards, the external temperature Tₒ and the internal temperature Tᵢ rise at the same rate, with the difference ΔT between them remaining unchanged.

At instant t₄, the external temperature reaches the desired maximum temperature of 250 °C. At this point, the raising of the temperature is stopped and this level of the external temperature is maintained. The internal temperature continues co rise, reaching the external temperature at instant t₅. The heat treatment of the timber is continued at this maximum temperature of 250 °C until instant t₆, whereupon the lowering of the external temperature is started. The internal temperature follows the external temperature with a certain time delay, and the external temperature is lowered in a steady and linear fashion so that the temperature difference ΔT between the internal and external temperatures is the same as when the temperature was being raised. The temperatures are lowered steadily down to the heat treatment threshold of 140 °C, at which point the heat treatment of the timber has been completed.

The essential point in this embodiment is that the graphs representing the rise and fall in the temperature are mainly mirror images of each other, in other words, the absolute value of the difference between the internal and external temperatures is of equal magnitude in the same temperature range during heating and cooling. Moreover, in the embodiment described, this difference is constant for most of the time during the process. As the heating and cooling phases are equal in duration, every part of the timber is at the same temperature, i.e. subject to the same kind of temperature changes, for a substantially equal length of time.

In the embodiment described above, before the heat treatment, the timber has been dried at a high temperature of over 100 °C, so the initial impulse S that gives the process a fast start occurs above the heat treatment threshold of 140 °C. But if the initial temperature of the timber is relatively low, i.e. clearly below the heat treatment threshold, then the initial impulse and the levelling of the temperature difference can be effected below the heat treatment threshold. In this case, the graphs representing the rise and fall in the cemperature are even more exact mirror images of each other.

In the foregoing, the invention has been described by way of example by the aid of the attached drawing while different embodiments of the invention are possible within the framework of the inventive idea defined by the claims.

## Claims

1. Procedure for heat treatment of timber, in which procedure the timber is dried to a humidity level below 15 %, whereupon the temperature of the timber is raised above a heat treatment threshold above which the desired changes produced by the heat treatment begin to appear, the timber is kept at the required temperature for as long as is necessary for the treatment, the temperature of the timber is lowered below the heat treatment threshold, and above the heat treatment threshold, both when the temperature is being raised and when it is being lowered, the difference between the internal and external temperatures of the timber is kept within certain limits, **characterised** in that, above the heat treatment threshold, the heating and cooling phases are of equal duration and the absolute value of the difference between the internal and external temperatures is maintained at a substantially equal magnitude at temperatures corresponding to each other during heating and cooling so that every part of the timber is at the same temperature for a substantially equal length of time.

2. Procedure as defined in claim 1 **characterised** in that the temperatures are raised and lowered in a linear manner.

3. Procedure as defined in claim 1 or 2 **characterised** in that the temperature difference is kept constant for a substantial part of the time during which the temperature is being raised or lowered.

4. Procedure as defined in claim 1 or 2 **characterised** in that the temperature difference is changed as a function of temperature.

5. Procedure as defined in any one of claims 1 - 4, **characterised** in that the timber is dried to a humidity below 10, preferably below 5 %.

6. Procedure as defined in any one of claims 1 - 5, **characterised** in that the heat treatment threshold is about 140 °C.

7. Procedure as defined in any one of claims 1 - 6, **characterised** in that, during the heat treatment, the temperature of the timber is raised to a level in the range 150 - 200 °C to increase the strength, surface hardness, flexural resistance and elastic flexural strength of the timber.

8. Procedure as defined in any one of claims 1 - 6, **characterised** in that, during the heat treatment, the temperature of the timber is raised to a level in the range 200 - 300 °C to improve the rot resistance properties of the timber.

9. Procedure as defined in any one of claims 1 - 8, **characterised** in that the heat treatment is carried out in a substantially non-pressurised room.

## Patentansprüche

1. Verfahren zur Wännebehandhmg von Holz, bei welchem Verfahren das Holz auf einen Feuchtigkeitspegel unter 15 % getrocknet wird, woraufhin die Temperatur des Holzes über einen Wärmebehandlungsschwellwert erhöht wird, über dem die von der Wärmebehandlung hervorgerufenen, erwünschten Änderungen beginnen aufzutreten, das Holz auf einer erforderlichen Temperatur so lange wie es für die Behandlung notwendig ist, gehalten wird, die Temperatur des Holzes unter den Wärmebehandlungsschwellwert abgesenkt wird und über dem Wännebehandlungsschwellwert, sowohl wenn die Temperatur angehoben wird, als auch wenn sie abgesenkt wird, der Unterschied zwischen der inneren und äußeren Temperatur des Holzes innerhalb bestimmter Grenzen gehalten wird,
dadurch gekennzeichnet, daß oberhalb des Wärmebehandlungsschwellwertes die Aufhei2- und Abkühlphasen gleiche Dauer haben und der Absolutwert des Unterschiedes zwischen der inneren und der äußeren Temperatur während des Aufheizens und Abkühlens bei sich entsprechenden Temperaturen auf einer im wesentlichen gleichen Größe gehalten wird, so daß jeder Teil des Holzes für eine im wesentlichen gleich lange Zeitdauer auf der gleichen Temperatur ist.

2. Verfahren nach Anspruch 1, dadurch gekennzeichnet, daß die Temperaturen linear erhöht und abgesenkt werden.

3. Verfahren nach Anspruch 1 oder 2, dadurch gekennzeichnet, daß der Temperaturunterschied für einen wesentlichen Teil der Zeitdauer konstant gehalten wird, während der die Temperatur angehoben oder abgesenkt wird.

4. Verfahren nach Anspruch 1 oder 2, dadurch gekennzeichnet, daß der Temperaturunterschied als eine Funktion der Temperatur geändert wird.

5. Verfahren nach einem der Amprüche 1 bis 4, dadurch gekennzeichnet, daß das Holz auf eine Feuchtigkeit unter 10, vorzugsweise unter 5 % getrocknet wird.

6. Verfahren nach einem der Ansprüche 1 bis 5, dadurch gekennzeichnet, daß der Wärmebehandlungsschwellwert etwa 140 °C beträgt.

7. Verfahren nach einem der Ansprüche 1 bis 6, dadurch gekennzeichnet, daß während der Wärmebehandlung die Temperatur des Holzes auf einen Pegel im Bereich 150 bis 200 °C angehoben wird, um die Festigkeit, Oberflächenhärte, den Biegewiderstand und die elastische Biegefestigkeit des Holzes zu erhöhen.

8. Verfahren nach einem der Ansprüche 1 bis 6, dadurch gekennzeichnet, daß während der Wärmebehandlung die Temperatur des Holzes auf einen Pegel im Bereich 200 bis 300 °C erhöht wird, um die Fäulniswiderstandseigenschaften des Holzes zu verbessern.

9. Verfahren nach einem der Ansprüche 1 bis 8, dadurch gekennzeichnet, daß die Wärmebehandlung in einem im wesentlichen nicht unter Druck gesetzten Raum durchgeführt wird.

## Revendications

1. Procédé de traitement thermique du bois de construction, procédé dans lequel on sèche le bois de construction jusqu'à un niveau d'humidité inférieur à 15 %, à la suite de quoi on élève la température du bois au-dessus d'un seuil de traitement thermique au-dessus duquel les changements désirés produits par le traitement thermique commencent à apparaître, on maintient le bois à la température requise aussi longtemps que nécessaire pour le traitement, on diminue la température du bois jusqu'en-dessous du seuil de traitement thermique, et alors que l'on se trouve au-dessus du seuil de traitement thermique à la fois lorsque l'on élève la température et qu'on la diminue, on maintient dans certaines limites la différence entre les températures intérieures et extérieures du bois, caractérisé en ce que, au-dessus du seuil de traitement thermique, les phases de chauffage et de refroidissement sont de même durée et on maintient la valeur absolue de la différence entre les températures internes et externes à une valeur sensiblement égale pour des températures qui se correspondent mutuellement pendant le chauffage et le refroidissement de sorte que chaque partie du bois est à une même température pour une durée sensiblement égale.

2. Procédé selon la revendication 1, caractérisé en ce que l'on élève et on diminue les températures linéairement.

3. Procédé selon la revendication 1 ou 2, caractérisé en ce qu'on maintient constante la différence de température pendant une partie substantielle du temps durant lequel on élève et l'on diminue la température.

4. Procédé selon la revendication 1 ou 2, caractérisé en ce qu'on modifie la différence de température en fonction de la température.

5. Procédé selon l'une quelconque des revendications 1 à 4, caractérisé en ce qu'on sèche le bois jusqu'à une humidité inférieure à 10, de préférence inférieure à 5 %.

6. Procédé selon l'une quelconque des revendications 1 à 5, caractérisé en ce que le seuil de traitement thermique est d'environ 140 ° C.

7. Procédé selon l'une des revendications 1 à 6, caractérisé en ce que pendant le traitement thermique, on élève la température du bois à un niveau de l'ordre de 150 à 200 ° C pour accroître la résistance, la dureté superficielle, la résistance à la flexion et la rigidité en flexion élastique du bois.

8. Procédé selon l'une des revendications 1 à 6, caractérisé en ce que pendant le traitement thermique, on élève la température du bois à un niveau de l'ordre de 200 à 300 ° C pour améliorer les propriétés de résistance à la putréfaction du bois.

9. Procédé selon l'une quelconque des revendications 1 à 8, caractérisé en ce qu'on mène le traitement thermique dans une salle sensiblement non pressurisée.
